

Nov. 16, 1937.

H. C. AVERY

2,099,093

ROOF COMPOSITION AND METHOD OF PRODUCING THE SAME

Original Filed March 28, 1932

Fig. 1.



Fig. 2.



Fig. 3.



Witness:

Stephen P. Peabody

Inventor:  
Henry C. Avery,  
By Frank L. Billenap  
Atty.

## UNITED STATES PATENT OFFICE

2,099,093

ROOF COMPOSITION AND METHOD OF  
PRODUCING THE SAME

Henry C. Avery, New Brunswick, N. J., assignor,  
by mesne assignments, to The Patent and Li-  
censing Corporation, New York, N. Y., a cor-  
poration of Massachusetts

Application March 28, 1932, Serial No. 601,702  
Renewed June 25, 1935

4 Claims. (CL. 91—70)

This application is a continuation in part of my application Serial No. 256,862, filed February 25, 1928.

This invention relates to composition roofing and has more particular reference to an improved asphaltic roofing material and a method of producing the same. My invention finds one particular adaptation in that type of roofing which consists of a felted foundation of fibrous material, such as rag or asbestos or similar fibres formed into a sheet on a paper making machine, and converted into material suitable for use as roofing by saturating the felted sheet with a waterproof saturant such as molten asphalt, and then coating on one or both faces thereof, with waterproof and weatherproof material such as blown asphalt. This coating material is usually spread upon the sheet in a layer of sufficient thickness to provide a barrier to the entrance of moisture into the pore spaces of the sheet, and to otherwise protect the sheet against the influence of the elements. As already indicated, one of the important functions of the layer of coating material, is to prevent the absorption of moisture by the sheet, since the absorption of moisture renders the material liable to deterioration upon exposure to the changing weather conditions, by virtue of the fact that the absorbed moisture tends to swell or bulk the felted base and cause disintegration thereof under the changing weather conditions. It is important that the layer of coating material should preserve its flexibility and ductility as long as possible and retain its integrity so as to properly protect the sheet against the entrance of moisture thereinto, and otherwise enable the coating layer to perform its protective functions.

The coating layer applied to the face of the sheet which will normally constitute the exposed surface of the roofing material may have imbedded therein a layer of grit or crushed mineral or any suitable form such as crushed slate or the like, the purpose of which is to provide a masking layer of wear and weather resistant material for the waterproof coating, and to impart to the roofing material any desired ornamental color effects. From a sheet thus prepared, there may be then cut the roofing shingles or shingle strips in the form in which they are to be applied on the roof or the sheet may be formed into rolls and applied as roll roofing.

I have heretofore referred to the necessity for covering the felted base of this type of roofing with a layer of coating material of sufficient thickness so as to afford at all times adequate protec-

tion for the felted base. I have observed that in the prepared roofing as produced under present day commercial operation, the coating layer is in time affected by the action of atmospheric conditions normally existing in actual use to such an extent that ultimately it ceases to provide the necessary protection to the roofing base. While the material which is usually employed as the coating for the roofing base is generally a blown asphalt having a melting point of about 10 220 degrees F., I have found that nevertheless the atmospheric conditions to which the roofing material is sometimes subjected, are sufficient to induce what appears to be a very slow and irregular internal flow of the coating material, 15 the nature and extent of which varies with the varying weathering conditions to which the material may be subjected. Apparently under the influence of the solar rays and sometimes also under the action of the excessive temperatures 20 of the roof-supporting structure, there is caused more or less internal flow of the coating material in various directions and in irregular degree, due apparently to the polymerization and surface hardening and shrinkage of the exposed coating layer induced by the normal 25 weathering effects. The slipping of the polymerized and hardened surface layer over the softer and yet unaffected portion of the coating layer, causes the former to crack and the softer portions to flow into the cracks thus produced. It will be appreciated, of course, that this flow and the displacement of the harder material by the softer, is indeed imperceptibly slow and can be observed only upon examination of the coating 30 layer over considerable periods of time. It is a fact, nevertheless, that this flow does occur and proceeds continually, with the formation, as a result thereof, of numerous ridges or crests and furrows or valleys distributed in irregular fashion over the surface of the roofing base, and ordinarily giving a crazed or checked appearance thereto. These formations, which I believe to be due to the aforesaid occurrence of internal 35 flow, may be readily noted upon examination of 40 roofing material of this character which has been exposed on a roof for a considerable length of time, during which it has had an opportunity of being subjected to one or more normal cycles of changing weather conditions. Manifestly 45 these formations detract from the protective properties of the coating layer, since the continuance of this action ultimately results in hardening of the coating to such an extent that the material becomes brittle, and the cracks formed 50 55

as above described, or by the movement of the roofing base under the action of wind and local expansion and contraction, give access of moisture to the roofing base and otherwise expose the base to rapid deterioration.

5 These difficulties cannot usually be avoided by employing a layer of greater thickness or of a thickness in excess of the usual optimum thickness which ranges from .025 to .060 of an inch, 10 since a layer of asphalt which is too thick is liable to crack from stresses set up by unequal heat and cooling, especially in winter weather when the coating asphalt becomes unusually hard and brittle.

15 By my present invention I provide a method whereby the foregoing difficulties may be eliminated. In accordance therewith, I combine with the ordinary layer of coating material applied to the sheet in the manufacture thereof, an additional layer of material which is itself highly 20 water resistant and also capable of resisting to the utmost any tendency for internal flow to take place therein and which furthermore prevents the internal flow, from taking place in the layer of asphalt thereunder. In this way the combined 25 layer permanently retains the desirable uniform thickness and avoids the production of checking and crazing on the exposed surface thereof, such as occurs in the roofing products of this type as 30 now produced.

In carrying out my invention I employ in conjunction with the ordinary layer of coating asphalt a relatively thin overlying layer or film of a dispersion of waterproofing material. In order 35 to effectuate the purposes of my present invention, the dispersion layer must be of a non-drying base such as asphalt, and the dispersed base should preferably be softer than the underlying coating layer. The dispersion is one which upon 40 the removal of the water and the coalescence of the dispersed particles assumes a structure rendering it capable of resisting flow at temperatures greatly in excess of the fusing or melting point of the dispersed asphalt. Dispersions of asphalt 45 having the aforesaid property of drying to a relatively infusible film, may be produced in various ways, although I prefer to employ for this purpose a dispersion of asphalt of a melting point ranging from 100 to 170 degrees F., made as described in 50 the patent to Lester Kirschbraun No. 1,620,900. Asphalt dispersions made in accordance with the Kirschbraun process are capable of drying to a film of substantial smoothness, the weathering of the film proceeding uniformly and without any 55 checking or crazing of the film. By providing a film of sufficient thickness, the weathering action is only superficial and does not affect the entire depth of the film. When a dispersion of this character is superposed upon a layer of asphalt 60 and the water is driven off or otherwise removed therefrom, it forms with the subjacent layer of asphalt an inseparable structure. In this structure, the outer layer of coalesced asphalt provides the requisite waterproofing and weather- 65 proofing qualities and by virtue of the peculiar physical structure of this composition it is itself completely stable to internal flow and furthermore prevents the occurrence of internal flow in the subjacent layer, or in any case prevents such 70 internal flow from affecting the uniform thickness of the composite layer and evidencing itself in the form of cracks and checks on the outermost surface thereof. Furthermore, because of the flexibility and ductility of the softer asphalt used 75 in producing the dispersion films of this type and

the inability of the films to undergo internal movement, they remain substantially unaffected by extreme conditions of temperature, and no cracking of the outer surface of the composite layer results under such conditions, and the resistance to the destructive action of the weather is thereby greatly prolonged. In order to increase the opacity of the dispersion film, as well as for other desired effects, suitable fibrous or granular fillers may be combined with the dispersion.

The principle of my invention as heretofore described may be utilized with advantage in the production of roofing having other than a felted fibrous base, and protected with an asphaltic 15 layer. Thus in accordance herewith, the composite layer of asphalt surmounted by a layer of asphalt dispersion may be applied to metallic, and wooden roofing bases, as well as to bases composed of various moulded compositions such 20 as cement and the like, or even to bases composed of moulded compositions of asphalt and fiber or other filler.

In the accompanying drawing, the several views are enlarged cross-sections of roofing material which may be produced in accordance with my invention.

In these views, numeral 1 indicates the roofing base which may be a felted sheet, or any other 30 desirable base, such as metal, wood, or a moulded composition. At 2 is indicated the layer of coating which may be applied in any convenient manner to the base after the formation thereof. The numeral 3 is intended to indicate the layer of 35 coalesced asphalt.

In Figure 1, the layer of coalesced asphalt 3 provides the finish coat for the roofing and this construction is particularly suitable for the production of a felt base product similar to the "rubber roofing" of commerce, and having no 40 surfacing material in the outermost layer.

In Figure 2, the layer 3 may have imbedded therein a surfacing material 4 such as crushed slate or the like.

In the form shown in Figure 3, the asphalt layer may have fine grit 5, such as talc or mica imbedded therein, and the layer 3 of asphalt dispersion is superposed upon the layer of fine grit so as to completely fill the interstices therebetween and form a coalesced asphalt layer of 50 desired thickness firmly united to the subjacent layers. If desired, talc or similar surfacing material may be applied over the layer 3 of coalesced asphalt in the construction illustrated in 55 Figure 3.

In producing roofing material having a felted fibrous foundation in accordance with my invention, the usual manner of saturating the felt base sheet may be followed and after the sheet has been withdrawn from the saturating apparatus and the saturant on the surfaces of the sheet has been absorbed into the pores thereof, the sheet is then conducted to the usual coating rolls where coating asphalt, as for example a 220 degree F. melting point blown asphalt is applied thereto. The thickness of this coating layer may be substantially the same as is common in the industry, but by suitably adjusting the coating rolls the thickness of the coating may be varied as desired, so as to produce a thinner layer than the usual coating layer of asphalt. Before this layer of molten asphalt has cooled, there is then applied thereover the dispersed asphalt so as to produce a layer of asphalt dispersion of uniform thickness overlying the rela- 76 78

tively hot soft layer of asphalt. In order that the weathering of the resultant film shall be superficial only and not affect its entire depth, the dispersion layer should be regulated in thickness 5 from 0.020 to 0.030 of an inch. The asphalt dispersion may be applied in any convenient way as by means of a spray or the like. As the sheet progresses in its travel, the heat from the coated base will assist in the evaporation of the water 10 from the layer of asphalt dispersion. Where it is desired to apply mineral surfacing the sheet may be fed along until the dispersion layer assumes a substantial degree of tackiness, so that the surfacing material may be applied and pressed by 15 suitable rolls into intimate contact with the tacky layer of the asphalt dispersion. As the water becomes completely removed from the dispersion layer, the particles thereof coalesce and at the same time the underlying layer of asphalt cools 20 sufficiently to cause it to harden, the layer of coalesced asphalt thus becoming united into an inseparable structure with the hardened layer of asphalt.

In some cases the opposite surface of the sheet 25 may also be provided with a coating layer of asphalt and in such case, this layer may also have applied thereto an overlying layer of asphalt dispersion similar to the layer 3.

The foregoing method may, if desired, be modified 30 by delaying the application of the asphalt dispersion to the coated sheet until the layer of the coating asphalt has cooled and solidified. This may be readily accomplished without entailing the loss of a great deal of time, inasmuch 35 as the coating material generally employed has a substantially high melting point, so that by conducting the sheet with the layer of asphalt thereon through the atmosphere for a relatively short distance, this layer will very quickly congeal and harden. If desired, the cooling of the 40 asphalt layer and the solidification thereof may be assisted by directing a blast of cool air upon the coated sheet, prior to the application of the asphalt dispersion, and similar means may also be employed if desired to assist the removal of 45 water from the dispersion layer to enable the latter to more quickly dry and harden or reach an adhesive and tacky condition suitable for the application of the surfacing material thereto, where surfacing material is to be applied.

For certain purposes particularly where the roofing is to be used on a cheaper type of building structure, it is desirable sometimes, for purposes of economy, to omit the granular surfacing 55 material and to finish the roofing with a coating of colored material to impart to the roof at least some degree of ornamentation. In producing roofing material of this class, in accordance with my invention I employ for the dispersion layer to 60 be applied over the ordinary asphalt coating, a dispersion of colorable waterproof pitch, or the like which as before stated is of a non-drying base, softer than the underlying coating and approximately of the same characteristics as the dispersion films applied as previously described. The dispersion of this material may be formed in accordance with the processes described in 65 the said patent to Lester Kirschbraun, and the dispersed material may then have incorporated therein any desired coloring agent such as mineral pigment, or the like. The colored dispersion may then be applied to the sheet previously coated with asphalt, in accordance with any of the methods above described.

75 My invention is also adapted for building up a

structure in place upon a roof. For example, asphalt coated roofing in the form of rolls may be applied to the roof structure, the successive layers being cemented along the overlapping margins thereof in the well known manner, and thereafter the sheets may be covered with a layer of the dispersion, the latter being either sprayed or brushed onto the surface and then permitted to dry and harden, and form the composite layer with the coating material of the roofing base as 10 already described. Obviously, mineral or similar surfacing material may, if desired, be distributed in any suitable way in the outermost layer of dispersion, before the latter has completely hardened.

15 It will be noted that in all the forms in which my invention may be embodied, I provide a composite coating layer, the outermost portions of which comprises an infusible structure which serves to prevent rapid deterioration of the fresh 20 and intact subjacent stratum or asphalt or similar coating substance.

25 It will be apparent that while I have described my invention in connection with roofing, I do not mean to be restricted thereto, as obviously, many other surfaces which are subjected in use to weathering conditions and similar destructive action may be protected and their resistance to such destructive influences may be prolonged by coating the same with a composite layer in accordance with the methods I have herein described.

30 It is another advantage of my invention that when a relatively thin asphalt coating is applied in connection with a superposed, relatively thin film of emulsion, as hereinabove disclosed, the grit may be forced through the film of emulsion so that the lower portions of the grit particles become partially embedded in the layer of molten asphalt before the same has congealed. Thereafter, when the under layer of molten asphalt has 35 set and the film of emulsion has coalesced, the grit will be anchored both by the asphalt layer and the coalesced emulsion layer, thus offering a 40 secure anchorage for the grit.

45 What I claim is:

1. The method of making roofing of the character described which comprises coating a roofing base with molten bituminous waterproofing material having a relatively high melting point, applying to the coated sheet a secondary coating 50 of bituminous waterproofing material of relatively low melting point dispersed in an aqueous medium, while the first named coating is at an elevated temperature whereby to effect a heat interchange between said coatings, and permitting 55 the secondary coating to dry and become united with the first named coating.

2. The method of making roofing material of the character described which comprises coating a saturated sheet of roofing base with molten 60 waterproofing substance, and substantially immediately thereafter applying to the coated sheet a secondary coating of non-fluid bitumen dispersed in an aqueous medium, and embedding in said secondary coating while the same is in a 65 soft and tacky condition, comminuted surfacing material.

3. The method of making roofing of the character described which comprises coating a roofing base with a thin layer of bituminous waterproofing material, applying to the coated sheet a secondary coating of relatively thin bituminous waterproofing material dispersed in an aqueous medium, applying grit to the sheet, while the 70 bituminous waterproofing material is molten and 75

before the dispersion has coalesced, and embedding the grit in both coatings and permitting the coatings to dry and become united whereby to anchor the grit to both coatings.

5. 4. The method of making material of the character described which comprises coating a saturated sheet of a roofing base with a thin film of molten asphalt, substantially immediately there-

after applying to the coated sheet a secondary coating of asphalt dispersed in an aqueous medium, applying grit to and embedding the same in both coatings and permitting the secondary coating to dry and become united with the first 5 named coating.

**HENRY C. AVERY.**